

## UNITED STATES PATENT OFFICE.

WILLIAM BENJAMIN GERO, OF BLOOMFIELD, NEW JERSEY, ASSIGNOR TO WESTINGHOUSE LAMP COMPANY, A CORPORATION OF PENNSYLVANIA.

## SEAL FOR HARD GLASS.

No Drawing.

Application filed July 28, 1926. Serial No. 125,591.

The present invention relates to a novel metallic seal for evacuated containers composed of hard glass, and it involves the use of an alloy of tungsten and molybdenum.

5 It has been proposed to employ molybdenum or tungsten as seals for evacuated containers consisting of hard or silica glass. I have discovered that an alloy of these metals in suitable proportion may be employed for 10 this purpose.

Therefore, it is an object of my invention to provide a suitable seal for hard glass which combines certain of the advantages obtained by using molybdenum or tungsten separately.

15 Another object of the invention is to provide a seal for hard glass which may be readily varied with respect to its coefficient of expansion so as to make the same suitable for a great variety of glasses having different coefficients of expansion.

20 Other objects of the invention will become apparent as the following description is read.

Tungsten and molybdenum have been used quite extensively for sealing to glass, especially silicate glasses. In manufacturing a 25 tungsten seal it is customary to bead the metal several times if a straight-through seal is made, but in press work the second beading operation is not always essential. Beading 30 comprises slipping a glass tube over the metal wire and heating the glass and metal until the glass is fused to the metal. In making seals employing molybdenum it has been found preferable to employ the wrapping method 35 which consists in heating the molybdenum wire and applying thereto molten glass obtained from a cane or solid rod of glass. Molybdenum seals are found more desirable 40 if a straight-through seal is to be employed, whereas for press work the tungsten seal is better suited.

45 It is further evident that either molybdenum or tungsten alone does not furnish any wide range of expansion coefficients whereas by merely altering the proportions of the constituents of an alloy of tungsten and molybdenum a considerable range may be obtained which makes the alloy suitable for a variety of hard glasses having different coefficients of expansion. Tungsten has a coefficient of expansion from 0° C. to about 500° C. of from  $4.2 \times 10^{-6}$  to  $4.8 \times 10^{-6}$  respectively, and commercial molybdenum between

25° and 100° C. from  $4.6 \times 10^{-6}$  to  $5.4 \times 10^{-6}$  per degree centigrade, respectively, as determined by the Bureau of Standards.

55 Although it has been proposed to employ as a seal an alloy of iron and nickel, the composition of which can be varied to obtain different coefficients of expansion, such material alone is unsuitable for sealing purposes since it does not wet the glass and form an hermetic seal. Therefore, it is customary in using such an alloy in seals to combine therewith as a coating material a substance such as copper or platinum which wets the glass and seals thereto.

60 I have found that an alloy of tungsten and molybdenum possesses all of the desirable properties essential to the formation of an 65 hermetic seal and at the same time provides for obtaining a wide range of coefficients of expansion suitable for a number of different glasses having different coefficients of expansion.

70 A specific embodiment of the invention may comprise about 80% of tungsten and about 20% of molybdenum, although as indicated above, these proportions may be varied to suit special needs. If a wire having a high 75 coefficient of expansion is desired, the proportion of tungsten should be increased and vice versa if a lower coefficient of expansion is desired. Tungsten has a lower coefficient of expansion than molybdenum, therefore the 80 greater percentage of tungsten employed the 85 closer the coefficient of expansion of the alloy is to tungsten.

90 The specific alloy composition stated has been found to satisfactorily seal to a hard 95 glass known as G 702-P, such glass consisting of about 72% of silica ( $SiO_2$ ), 15% of boron oxide ( $B_2O_3$ ), 6.5% of lead oxide ( $PbO$ ) about 4.4% of sodium oxide ( $Na_2O$ ) and about 2% of aluminum oxide ( $Al_2O_3$ ). This 95 glass has a melting point of about 760° C. and a coefficient of expansion of about  $4.5 \times 10^{-6}$ .

100 The alloy may be prepared by mixing suitable proportions of the oxides of tungsten and molybdenum and reducing to metal by means of hydrogen in accordance with standard processes employed in the manufacture of tungsten. The metal powders may be employed directly without going through the reduction step. The powders of the metal 105 may then be agglomerated by pressing in

suitable molds and subjecting the pressed powders to heat treatment in hydrogen gas until they are sufficiently strong to permit handling. The sintered bars are then rendered dense and coherent by passage of an electric current therethrough, this latter operation being termed the treating step. The treated bar may then be mechanically worked to wire or filamentary sizes by hot-swaging and drawing, slightly lower temperatures than those employed for working tungsten being preferably employed. The entire process of sintering, treating and mechanical working is substantially like that employed in manufacturing tungsten with the exception that such modifications are resorted to as found essential because of the character of material undergoing treatment.

An alloy of tungsten thus formed may be employed as a leading-in wire for lamps, radio tubes, rectifiers and the like or may be utilized wherever it is desired to make an hermetic seal to hard glasses.

Modifications of the invention may occur to those skilled in the art, however, such modifications are contemplated by me as

come within the scope of the invention as defined in the appended claims.

What is claimed is:

1. In combination with a container consisting of hard glass, a conductor sealed therein and consisting of an alloy of tungsten and molybdenum.
2. The combination with a container consisting of a glass having a coefficient of expansion of about  $4.5 \times 10^{-6}$ , of a conductor sealed thereto consisting of an alloy of tungsten and molybdenum.
3. The combination with a container consisting of a glass having a coefficient of expansion of about  $4.5 \times 10^{-6}$ , of a conductor sealed thereto consisting of an alloy of tungsten and molybdenum in the proportion of about 80% and about 20%, respectively.
4. An electric appliance of the character described provided with a leading-in conductor composed of an alloy of tungsten and molybdenum sealed in hard glass.

In testimony whereof, I have hereunto subscribed my name this 27th day of July, 1926.

WILLIAM BENJAMIN GERO.